# EUROPEAN PATENT SPECIFICATION

(11) **EP 3 397 740 B1**
(45) Date of publication and mention of the grant of the patent: **08.12.2021**
(21) Application number: 16819121.1
(22) Date of filing: 27.12.2016
(51) Int. Cl.: C10M 169/04

(54) **LUBRICATING OIL COMPOSITION FOR DIESEL ENGINES**
SCHMIERÖLZUSAMMENSETZUNG FÜR DIESELMOTOREN
COMPOSITION D'HUILE LUBRIFIANTE POUR MOTEURS DIESEL

(30) Priority: 28.12.2015 JP 2015257263
(43) Date of publication of application: 07.11.2018
(73) Proprietor: Shell Internationale Research Maatschappij B.V., 2596 HR The Hague (NL)
(72) Inventor: UEDA, Mao, Kanagawa Aikou 243-0303 (JP); HANYUDA, Kiyoshi, Kanagawa Aikou 242-0303 (JP)
(74) Representative: Shell Legal Services IP
(86) International application number: PCT/EP2016/082719
(87) International publication number: WO 2017/114836

(56) References cited:
- EP-A1- 2 000 523
- EP-A1- 2 164 885
- EP-A1- 2 256 180
- WO-A1-2015/097152
- US-A1- 2014 106 998

## Description

### Field of the Invention

This invention relates to an engine oil for automobiles (lubricating oil composition for internal combustion engines), and more specifically relates to a lubricating oil composition for diesel engines with superior fuel efficiency, oil consumption control and detergency.

### Background of the Invention

One problem with crankcase lubricating oils is that the lubricating oil is liable to escape from the crankcase because of so-called blow-by gas. The blow-by gas, or gas/lubricating oil mixtures of this kind, are preferably recycled in the engine rather than being exhausted to the atmosphere. In some engines such recycling is carried out by injecting the blow-by gas into the engine's air-intake system so that the lubricating oil is combusted in the piston chambers. Recycling of the blow-by gas solves the problem of emissions but, on the other hand, there is the possibility that problems may arise in that deposits may form in the air-intake system. For example, if the deposits form in the air compressor, the compressor will not work properly and will even be prone to damage. As a further example, if an air cooler is present between the compressor and the cylinder block crankcase, the air cooler may become contaminated. There has been a demand for the provision of diesel engine systems that will prevent or reduce the formation of such deposits, see for example JP5501620.

At the same time, there has been a demand for lower fuel consumption. To achieve lower fuel consumption investigations have been carried out to manufacture compositions having the appropriate viscosity characteristics by using friction modifiers to contribute to friction reducing performance, and by using viscosity index improvers to bring about a reduction in churning resistance and to maintain an oil film at high temperatures while having low viscosity at low temperatures, as described in Japanese Laid-open Patent 2014-210844.

WO2015097152 discloses a lubricating composition for use in the crankcase of an engine comprising: (i) a base oil comprising at least one monoester or a mixture of monoesters, wherein said monoester or mixture of monoesters has a kinematic viscosity at 100°C of not more than 4 mm<2>/s, a viscosity index of at least 130 and a Noack evaporation loss of not more than 20 wt%; and (ii) polymeric viscosity index improvers selected from (a) one or more comb polymers; (b) a poly (meth) acrylate polymer having 1 to mol% of one or more specific (meth) acrylate structural units represented by the formula, wherein R<2> is a straight chain or branched hydrocarbon group having not less than 16 carbon atoms; (c) styrene-diene hydrogenated copolymers; and (d) mixtures thereof.

EP2256180 discloses a lubricating oil composition which comprises a base oil of lubricating oil having a kinematic viscosity of 3.5 to 10 mm<2> /s at 100°C and a viscosity index of 100 or greater and (a) an ethylene-α-olefin copolymer having a number-average molecular weight of 2,500 to 25,000 and/or (b) a polymethacrylate having a number-average molecular weight of 10,000 to 30,000, wherein a kinematic viscosity of the composition is 5.6 to 15.0 mm<2> /s at 100°C.

However, there has been nothing yet which achieves enough satisfaction in suppressing deposit formation, demonstrating fuel economy and maintaining performance over long periods. Also, it seems that in future the downsizing of commercial vehicles which are fitted with diesel engines by adding boosting devices will keep on advancing, and it may be expected that the thermal loads on engine oils will increase. However, there has been the problem that good volatility has not been achieved with the lubricating oil compositions of the prior art.

The purpose of this invention, therefore, is to offer a lubricating oil composition for use in diesel engines which, when used as an engine oil for vehicles, does have excellent volatility and engine cleaning properties as well as fuel economising performance.

### Summary of the Invention

By dint of intensive research, the inventors have discovered that it is possible to solve the aforementioned problems by blending a specified base oil and a specified viscosity index improver with a specified dispersant and detergent and thereby satisfying the specified viscosity grade, and have thus perfected this invention. Specifically the invention is as follows.
Aspect (I) of the invention is a lubricating oil composition for diesel engines characterised in that it contains:
   a) a GTL base oil with a kinematic viscosity at 100°C of 4.5 to 5.5 mm²/s, consisting of either a single GTL base oil with a kinematic viscosity at 100°C of 4.5 to 5.5 mm <2> /s or a mixture of i) a GTL base oil with a kinematic viscosity at 100°C of 3.0 to 6.0 mm <2> /s; and ii) a GTL base oil with a kinematic viscosity at 100°C of 7.0 to 13 mm <2> /s,
   b) a comb-like PMA (polymethacrylate) based viscosity index improver and
   c) a boron-containing dispersant and boron-containing detergent, wherein the total amount of boron-containing dispersant and/or boron-containing detergent incorporated in terms of conversion to boron content relative to the total amount of the composition being not less than 0.025 mass% and not more than 0.050 mass%,
   wherein it satisfies 0W-30 or 5W-30 in the SAE J300 standard.
Aspect (II) of the invention is a lubricating oil composition for diesel engines in accordance with Aspect (I) which also includes a non-comb-like PMA (polymethacrylate) based viscosity index improver and an SCP (styrene-diene copolymer) based viscosity index improver and/or an OCP (olefin copolymer) based viscosity index improver and which further satisfies at least one of the following (1) to (3), the polymer amounts being minus diluents.
   (1) Non-comb-like PMA based viscosity index improver content/total viscosity index improver content (polymer having weight-average molecular weight of not less than 50,000): not more than 0.7
   (2) OCP based viscosity index improver content/total viscosity index improver content (polymer having weight-average molecular weight of not less than 50,000): not more than 0.2
   (3) SCP based viscosity index improver content/total viscosity index improver content (polymer having weight-average molecular weight of not less than 50,000): not more than 0.3
Aspect (III) of the invention is a lubricating oil composition for diesel engines in accordance with Aspect (I) or (II) satisfying the following viscosity characteristic. $\frac{\left[\begin{matrix}HTHS 100 ° C viscosity \left(capillary method\right) - \\ HTHS 100 ° C viscosity \left(TBS method\right)\end{matrix}\right]}{HTHS 100 ° C viscosity \left(TBS method\right)} = 0.07 to 0.15$ wherein HTHS 100°C viscosity (capillary method) is measured according to ASTM D5481 test method and the HTHS 100°C viscosity (TBS method) is measured according to ASTM D4683.

According to this invention, it is possible to offer a lubricating oil composition for use in diesel engines which, when used as an engine oil for vehicles, has excellent volatility and engine cleaning properties as well as fuel economising performance.

### Detailed Description of the Invention

The constituents (constituent elements), composition (contents of each constituent) and physical characteristics of the lubricating oil composition for diesel engines relating to this invention are described below, but the invention is in no way limited by these.

The lubricating oil composition of the present embodiment contains a GTL base oil as the base oil, a comb-like PMA based viscosity index improver and a boron-containing dispersant and a boron-containing detergent, and other constituents where necessary.

GTL (gas-to-liquid) oils synthesised by the Fischer-Tropsch process in the technology for liquefying fuels from natural gas are used as the base oil for the lubricating oil composition of this invention. Using such base oils makes it possible, in the framework of this invention, to improve oxidative stability as well as reducing evaporative losses.

When using comb-like polymers, in comparison with Yubase base oils it is possible to improve fuel consumption by using GTL base oils because, especially within the framework of this invention, the temporary shear viscosity at 100°C falls.

In particular, in this invention a GTL base oil having a kinematic viscosity at 100°C of 4.5 to 5.5. mm²/s is used. If the kinematic viscosity at 100°C of the base oil falls below 4.5, satisfactory volatility is not obtained. If the kinematic viscosity at 100°C exceeds 5.5, satisfactory fuel economy is not obtained.

Here, in order to obtain a base oil where the kinematic viscosity at 100°C is 4.5 to 5.5 mm²/s, it is preferable if it is a single GTL base oil with a kinematic viscosity at 100°C of 4.5 to 5.5 mm²/s, but in the case of manufacture it is suitable to mix two kinds, a GTL base oil (a1) where the kinematic viscosity at 100°C is 3.0 to 6.0 mm²/s and a GTL base oil (a2) where the kinematic viscosity at 100°C is 7.0 to 13 mm²/s. If the kinematic viscosity at 100°C of the low viscosity base oil constituent (a1) is below 3.0 mm²/s, the amount of evaporation increases, and it becomes difficult to maintain the viscosity of the composition over long periods. If using a high viscosity base oil constituent (a2) where the kinematic viscosity at 100°C exceeds 13 mm²/s, the low temperature viscosity at -40°C increases and low-temperature startability worsens. Furthermore, in this case, the ideal viscosity index of the mixed GTL base oil is 120 to 180, but 120 to 150 is even better.

For these GTL base oils a total sulphur content of less than 10 ppm is typically ideal, and a total nitrogen content of less than 1 ppm is even better. One example of such a GTL base oil product is Shell XHVI (trade name).

The lubricating oil of the present invention includes a boron-containing detergent as a detergent. There are no special restrictions for the boron-containing detergent, but mention may be made of boron-containing alkaline earth metal salts. More specifically, mention may be made of borated alkaline earth metal alkylsalicylate detergents and borated alkaline earth metal alkyl toluene sulphonate detergents. Borated calcium alkyltoluene sulphonate is ideal. Instances in the known art may be used for such boron-containing detergents (for example, borated alkaline earth metal alkyl toluene sulphonate detergents may be manufactured in accordance with Japanese Laid-open Patent 2008-297547) .

The lubricating oil composition of the present embodiment here may also include other detergents (for example, metallic detergents) so long as the effect of the invention is not impeded. As examples of metallic detergents, mention may be made of alkaline earth metal sulphonates, alkaline earth metal phenates, alkaline earth metal salicylates and alkaline earth metal naphthenates. As examples of the alkaline earth metals, mention may be made of calcium and magnesium. These may be used singly or in combinations of two or more kinds. Normally, use of sulphonates, phenates and salicylates of calcium or magnesium is preferred. For alkaline earth metal phenates it is preferable to use alkaline earth metal salts, especially calcium salts, of alkylphenols, alkylphenol sulphides and alkylphenol Mannich reaction products having straight-chain or branched alkyl groups of carbon number 4 to 30, but preferably 6 to 18. For alkaline earth metal salicylates it is preferable to use alkaline earth metals salts, and with special preference magnesium salts and/or calcium salts, of alkyl salicylic acids having straight-chain or branched alkyl groups of carbon number 1 to 30, but preferably 6 to 18. The base numbers of these may be freely chosen according to the type and purpose of the corresponding lubricating oil.

The lubricating oil composition of the present invention includes a boron-containing dispersant as a dispersant. For example, polybutenyl succinimide based dispersants, polybutenyl succinamide based dispersants, benzylamine based dispersants and succinate ester based dispersants may be borated.

Polybutenyl succinimides are obtained from polybutenes obtained by polymerisation of high-purity isobutene or mixtures of 1-butene and isobutene using a fluorinated boron based catalyst or an aluminium chloride based catalyst, and the products having a vinylidene structure at the terminals are normally contained in the amount of 5 to 100 mol%. From the standpoint of sludge-inhibiting effects, it is preferable to include 2 to 5, and in particular 3 to 4, nitrogen atoms in the polyalkylene-polyamine chains. Also, as polybutenyl succinimide derivatives, it is possible to use the so-called modified succinimides in which some or all of the amino and/or imino groups present have been neutralised or amidified by making boric acid compounds or oxygen-containing organic compounds such as alcohols, aldehydes, ketones, alkylphenols, cyclic carbonates and organic acids act on the aforementioned polybutenyl succinimide compounds.

The lubricating oil composition of the present invention is such as to contain any and at least one of the above mentioned boron-containing detergents and boron-containing dispersants together.

As examples of anti-wear agents imparting wear resistance and extreme-pressure resistance that can be used in the lubricating oil composition of the present embodiment, mention may be made of zinc dithiophosphates (ZnDTP). Typical examples of ZnDTP generally include zinc dialkyldithiophosphates, zinc diaryldithiophosphates and zinc arylalkyldithiophosphates. The alkyl groups here may be straight-chain or branched. For example, as regards the alkyl groups of the zinc dialkyldithiophosphates, zinc dialkyldithiophosphates having primary or secondary alkyl groups of carbon number 3 to 22 or alkylaryl groups substituted with alkyl groups of carbon number 3 to 18 may be used. As specific examples of zinc dialkyldithiophosphates, mention may be made of zinc dipropyldithiophosphate, zinc dibutyldithiophosphate, zinc dipentyldithiophosphate, zinc dihexyldithiophosphate, zinc diisopentyldithiophosphate, zinc diethylhexyldithiophosphate, zinc dioctyldithiophosphate, zinc dinonyldithiophosphate, zinc didecyldithiophosphate, zinc didodecyldithiophosphate, zinc dipropylphenyldithiophosphate, zinc dipentylphenyldithiophosphate, zinc dipropylmethylphenyldithiophosphate, zinc dinonylphenyldithiophosphate, zinc didodecylphenyldithiophosphate and zinc didodecylphenyl dithiophosphate.

The metal deactivators that can be used in the lubricating oil composition of the present embodiment include benzotriazoles and benzotriazole derivatives such as alkyl-tolyltriazoles, and benzimidazoles and benzimidazole derivatives such as tolimidazoles. Further examples are indazole derivatives such as tolylindazoles, benzothiazoles and benzothiazole derivatives such as tolylthiazoles. Mention may also be made of benzoxazole derivatives, thiadiazole derivatives and tolazole derivatives.

Examples of the anti-oxidants used in the lubricating oil composition of the present embodiment include amine-based anti-oxidants and phenol-based anti-oxidants. As examples of the aforementioned amine-based anti-oxidants, mention may be made of dialkyl-diphenylamines such as p,p'-dioctyl-diphenylamine (Nonflex OD-3, made by Seiko Chemical Ltd), p,p'-di-α-methylbenzyl-diphenylamine and N-p-butylphenyl-N-p'-octylphenylamine, monoalkyldiphenylamines such as mono-t-butyldiphenylamine and monooctyldiphenylamine, bis(dialkylphenyl)amines such as di(2,4-diethylphenyl)amine and di(2-ethyl-4-nonylphenyl)amine, alkylphenyl-1-naphthylamines such as octyl-phenyl-1-naphthylamine and N-t-dodecylphenyl-1-naphthylamine, 1-naphthylamine, aryl-naphthylamines such as phenyl-1-naphthylamine, phenyl-2-naphthylamine, N-hexylphenyl-2-naphthylamine and N-octylphenyl-2-naphthylamine, phenylenediamines such as N,N'-diisopropyl-p-phenylenediamine and N,N'-diphenyl-p-phenylenediamine, and phenothiazines such as Phenothiazine (made by Hodogaya Chemical Ltd.) and 3,7-dioctylphenothiazine. Phenol-based anti-oxidants include 2-t-butylphenol, 2-t-butyl-4-methylphenol, 2-t-butyl-5-methylphenol, 2,4-di-t-butylphenol, 2,4-dimethyl-6-t-butylphenol, 2-t-butyl-4-methoxyphenol, 3-t-butyl-4-methoxyphenol, 2,5-di-t-butylhydroquinone (Antage DBH, made by Kawaguchi Chemical Industry Co. Ltd.), 2,6-di-t-butylphenol, 2,6-di-t-butyl-4-alkylphenols such as 2,6-di-t-butyl-4-methylphenol and 2,6-di-t-butyl-4-ethylphenol, and 2,6-di-t-butyl-4-alkoxyphenols such as 2,6-di-t-butyl-4-methoxyphenol and 2,6-di-t-butyl-4-ethoxyphenol. Also, there are 3,5-di-t-butyl-4-hydroxybenzylmercapto-octylacetate, alkyl-3-(3,5-di-t-butyl-4-hydroxyphenyl) propionates such as n-octadecyl-3-(3,5-di-t-butyl-4-hydroxyphenyl) propionate (Yoshinox SS, made by Yoshitomi Fine Chemicals Ltd.), n-dodecyl-3-(3,5-di-t-butyl-4-hydroxyphenyl) propionate and 2'-ethylhexyl-3-(3,5-di-t-butyl-4-hydroxyphenyl) propionate, and benzenepropanoic acid 3,5-bis(1,1-dimethyl-ethyl)-4-hydroxy-C7~C9 side-chain alkyl ester (Irganox L135, made by Ciba Specialty Chemicals Ltd.), 2,6-di-t-butyl-α-dimethylamino-p-cresol, and 2,2'-methylenebis(4-alkyl-6-t-butylphenol)s such as 2,2'-methylenebis(4-methyl-6-t-butylphenol) (Antage W-400, made by Kawaguchi Chemical Industry Ltd.) and 2,2'-methylenebis(4-ethyl-6-t-butylphenol) (Antage W-500, made by Kawaguchi Chemical Industry Ltd). Furthermore, there are bisphenols such as 4,4'-butylidenebis(3-methyl-6-t-butylphenol) (Antage W-300, made by Kawaguchi Chemical Industry Ltd.), 4,4'-methylenebis(2,6-di-t-butylphenol) (Ionox 220AH, made by Shell Japan Ltd.), 4,4'-bis(2,6-di-t-butylphenol), 2,2-(di-p-hydroxyphenyl)propane (Bisphenol A, made by Shell Japan Ltd.), 2,2-bis(3,5-di-t-butyl-4-hydroxyphenyl)propane, 4,4'-cyclohexylidenebis(2,6-t-butylphenol), hexamethylene glycol bis[3-(3,5-di-t-butyl-4-hydroxyphenyl)propionate] (Irganox L109, made by Ciba Specialty Chemicals Ltd.), triethylene glycol bis[3-(3-t-butyl-4-hydroxy-5-methylphenyl)propionate] (Tominox 917, made by Yoshitomi Fine Chemicals Ltd.), 2,2'-thio-[diethyl-3-(3,5-di-t-butyl-4-hydroxyphenyl)propionate (Irganox L115, made by Ciba Specialty Chemicals Ltd.), 3,9-bis{1,1-dimethyl-2-[3-(3-t-butyl-4-hydroxy-5-methylphenyl) propionyloxy]ethyl} 2,4,8,10-tetraoxaspiro[5,5]undecane (Sumilizer GA80, made by Sumitomo Chemicals), 4,4'-thiobis(3-methyl-6-t-butylphenol) (Antage RC, made by Kawaguchi Chemical Industry Ltd.) and 2,2'-thiobis(4,6-di-t-butyl-resorcinol). Mention may also be made of polyphenols such as tetrakis[methylene-3-(3,5-di-t-butyl-4-hydroxyphenyl) propionate]methane (Irganox L101, made by Ciba Specialty Chemicals Ltd.), 1,1,3-tris(2-methyl-4-hydroxy-5-t-butylphenyl)butane (Yoshinox 930, made by Yoshitomi Fine Chemicals Ltd.), 1,3,5-trimethyl-2,4,6-tris(3,5-di-t-butyl-4-hydroxybenzyl)benzene (Ionox 330, made by Shell Japan Ltd.), bis-[3,3'-bis-(4'-hydroxy-3'-t-butylphenyl) butyric acid] glycol ester, 2-(3',5'-di-t-butyl-4-hydroxyphenyl) methyl-4-(2",4"-di-t-butyl-3"-hydroxyphenyl)methyl-6-t-butylphenol and 2,6,-bis(2'-hydroxy-3'-t-butyl-5'-methyl-benzyl)-4-methylphenol, and phenol-aldehyde condensates such as condensates of p-t-butylphenol and formaldehyde and condensates of p-t-butylphenol and acetaldehyde.

The lubricating oil composition of the present embodiment includes a comb-like polymethacrylate-based viscosity index improver. What is meant by a comb-like polymer is a polymer having a plurality of extended side chains in a comb form relative to the main polymer chain. The viscosity index improvers of the present embodiment include, among these comb-like polymers, viscosity index improvers which are comb-like polymethacrylate-based polymers. In this invention, what is meant by a "viscosity index improver" denotes a polymer having a weight average molecular weight of not less than 50,000.

Suitable instances of the comb-like polymethacrylate-based viscosity index improvers that may be used in the present embodiment are, for example, the polymers disclosed in Japanese Laid-open Patent 2010-532805.

Also, the comb-like polymethacrylate-based viscosity index improvers of the present embodiment ideally have a weight average molecular weight of 200,000 to 600,000, those of 250,000 to 500,000 are even better, and those of 300,00 to 450,000 are best of all. The PSSI (permanent shear stability index) is ideally not more than 10.

As specific examples of such comb-like polymethacrylate-based viscosity index improvers, mention may be made of Viscoplex 3-201 (registered trade mark) and Viscoplex 3-220 (registered trade mark).

The lubricating oil composition of the present embodiment may include viscosity index improvers other than comb-like polymethacrylate-based viscosity index improvers. As examples of such viscosity index improvers, mention may be made of one kind or more of polymers selected from the group comprising non-comb-like PMA (polymethacrylates), OCP (olefin copolymers) and SCP (styrene-diene copolymers).

For non-comb-like PMA (polymethacrylate)-based viscosity index improvers it is possible to use without any special restriction those known in the art, but those having a weight average molecular weight of 100,000 to 400,000 are ideal. Specific examples of such a PMA are those disclosed in Japanese Laid-open Patent 2014-125569.

For OCP (olefin copolymer)-based viscosity index improvers it is possible to use without any special restriction those known in the art, but those having a weight average molecular weight of 50,000 to 300,000 are ideal. Specific examples of such an OCP are those disclosed in Japanese Laid-open Patent 2014-125569.

For SCP (styrene-diene copolymer)-based viscosity index improvers it is possible to use without any special restriction those known in the art, but those having a weight average molecular weight of 200,000 to 1,000,000 are ideal. A specific example of such an SCP is Infineum (registered trade mark) SV150.

The lubricating oil composition of the present embodiment may contain polymers other than comb-like polymethacrylates as viscosity index improvers.

Such viscosity index improvers (polymers having a weight average molecular weight of not less than 50,000) are in general blended in a diluted state in a suitable liquid medium to make them easier to handle.

As examples of the defoamers that can be used in the lubricating oil composition of the present embodiment, mention may be made of organosilicates such as dimethylpolysiloxane, diethyl silicate and fluorosilicones and non-silicone based defoamers such as polyalkylacrylates.

The base oil content is ideally 60 to 90 mass% in terms of the total mass of the lubricating oil composition, but 65 to 90 mass% is better, and the range 70 to 85 mass% is better yet.

The content of viscosity index improvers (amount of viscosity index improvers as a whole) is not specially restricted and may be modified as appropriate. For example it may be 0.05 to 20 mass% in terms of the total mass of the lubricating oil composition. The ideal amounts of each of the various viscosity index improvers are given below.

There is no special restriction on the content of the comb-like PMA, but ideally it is 1.0 to 6.0 mass% in terms of the total amount of the lubricating oil composition, but 1.0 to 5.0 mass% is better and 1.0 to 4.0 mass% is best of all.

The non-comb-like PMA content is ideally such that non-comb-like PMA content / total viscosity index improver content is not more than 0.7.

The OCP content is ideally such that OCP content / total viscosity index improver content is not more than 0.2.

The SCP content is ideally such that SCP content / total viscosity index improver content is not more than 0.3.

If non-comb-like PMA (polymethacrylates), SCP (styrene-diene copolymers) and OCP (olefin copolymers) are included as viscosity index improvers, and these satisfy at least one (but ideally all) of the aforementioned ranges, it is possible within the framework of this invention to achieve the effects of the invention and also to reduce manufacturing costs.

In order to obtain the desired effect, the content of the boron-containing detergent and boron-containing dispersant must be not less than 0.025 mass% in terms of the boron content conversion value (total amount). The upper limit is not more than 0.050 mass%.

An explanation will be given of the ideal added amounts for other constituents which may be added to the lubricating oil composition of the present embodiment. First, the ideal added amount of anti-oxidants, individually or in combinations of plural kinds, will be in the range 0.01 to 2 mass% in terms of the total mass of the lubricating oil composition. The ideal added amount of metal deactivators, individually or in combinations of plural kinds, will be in the range 0.01 to 0.5 mass% in terms of the total mass of the lubricating oil composition. The ideal added amount of anti-wear agents (for example ZnDTP), individually or in combinations of plural kinds, will be, for example, in the range, as amount of phosphorus (P), 0.01 to 0.10 mass% but more preferably 0.05 to 0.08 mass% in terms of the total mass of the lubricating oil composition. The ideal added amount of defoamers, individually or in combinations of plural kinds, will be, for example, 0.0001 to 0.01 mass% in terms of the total mass of the lubricating composition. The ideal added amount of metallic detergents, individually or in combinations of plural kinds, will be, for example, 0.05 to 0.3 mass%, but more preferably 0.1 to 0.2 mass%, in terms of the total mass of the lubricating composition. The ideal added amount of ashless dispersants, individually or in combinations of plural kinds, will be, for example, be such as to present of the order of 0.01 to 0.3 mass% of nitrogen in terms of the total mass of the lubricating composition.

It is considered here that there is an excellent correlation between HTHS viscosity at 100°C and fuel consumption characteristics. There are various methods of measuring HTHS viscosity. Among them, there are cases where the viscosity obtained by measuring the HTHS viscosity by the capillary method and the viscosity measured by the TBS method differ, depending on the type of viscosity index improver used. Given that, to the extent that the value in Formula (1) below is large, the viscosity component as measured by the method using a capillary tube type viscometer (the capillary method) will be large, and the viscosity component as measured by using a rotational viscometer (TBS method) will be small, revealing that the difference between them will increase. In those cases, it denotes that the shear viscosity of the oil becomes smaller at sliding friction positions in situations close to such rotational viscometers between the crankshaft bearings. In other words, it is considered that it is possible to reduce the viscous resistance and to reduce the friction losses at the aforementioned positions. At the same time, at positions where the oil is subject to shear in situations close to a capillary viscometer, it is possible to maintain a high shear viscosity and thus satisfactory durability.

With the lubricating oil composition of the present embodiment, it was discovered that [(capillary viscosity - TBS viscosity) / TBS viscosity] satisfies 0.07 to 0.15, and in that connection low fuel consumption was manifested.

The method of measuring the capillary viscosity here is the value measured in accordance with the ASTM D5481 test method (150°C), taking the temperature condition at 100°C (shear velocity 1.0 * 10^6S⁻¹).

The method of measuring the TBS viscosity is the value measured by means of the method described in Japanese Patent 5565999.

### Examples

The invention is further explained next by means of examples of embodiment and comparative examples, but the invention is in no way limited by these examples.

The raw materials used in the examples of embodiment were as follows. The characteristics of the various base oils are shown in Table 1.

### Base Oils

- Base oil 1:XHVI 4 (GTL oil)
- Base oil 2:XHVI 8 (GTL oil)
- Base oil 3:XHVI 3 (GTL oil)
- Base oil 4:Yubase 4 (mineral oil)
- Base oil 5:Yubase 8 (mineral oil)
- Base oil 6:Yubase 3 (mineral oil)

### Additives Packages

DH-2 DI package 1: As shown in the tables, in the examples of embodiment when 14.00% was added, the boron content of the lubricating oil became 0.033 mass% {including boron-containing dispersant (borated calcium alkyltoluene sulphonate) and boron-containing detergent (borated succinate ester-based dispersant), and amount of other additives same as DI packages 2 and 3}

DH-2 DI package 2: As shown in the tables, in the examples of embodiment when 14.00% was added, the boron content of the lubricating oil became 0.027 mass% {including boron-containing dispersant (borated calcium alkyltoluene sulphonate) and boron-containing detergent (borated succinate ester-based dispersant), and amount of other additives same as DI packages 1 and 3}

DH-2 DI package 3: As shown in the tables, in the examples of embodiment when 14.00% was added, the boron content of the lubricating oil became 0.020 mass% {including boron-containing dispersant (borated calcium alkyltoluene sulphonate) and boron-containing detergent (borated succinate ester-based dispersant), and amount of other additives same as DI packages 1 and 2}

### Viscosity Index Improvers

- Viscosity index improver solution 1: Solution containing Viscoplex 3-220 (comb-like PMA-based viscosity index improver) (approx. 40% dilution)
- Viscosity index improver solution 2: Solution containing Viscoplex 3-201 (comb-like PMA-based viscosity index improver) (approx. 60% dilution)

• Viscosity index improver solution 3: Solution containing Viscoplex 6-954 (non-comb-like PMA-based viscosity index improver) (approx. 40% dilution)
• Viscosity index improver solution 4: Solution containing Lz7177B (olefin copolymer -based viscosity index improver) (approx. 87.5% dilution)
• Viscosity index improver solution 5: Solution containing Infineum (registered trade mark) SV150 (styrene-diene copolymer-based viscosity index improver) (approx. 93.5% dilution) Defoamer
• DCF 3 mass% solution

**Table 1**

| Base oil name | Base oil 1 | Base oil 2 | Base oil 3 | Base oil 4 | Base oil 5 | Base oil 6 |
|---|---|---|---|---|---|---|
| API category | Group 3 | Group 3 | Group 2 | Group 3 | Group 3 | Group 2 |
| Kinematic viscosity | | | | | | |
| @ 100°C mm2/s | 4.1 | 7.6 | 2.7 | 4.2 | 7.6 | 3.1 |
| @ 40°C mm2/s | 17.9 | 43.7 | 9.9 | 19.3 | 46.6 | 12.4 |
| Viscosity index JIS K 2283 | 130 | 143 | 112 | 125 | 129 | 10.4 |
| Noack evaporative loss mass% ASTM D5800 | 13.2 | 4.6 | 42.5 | 14.8 | 5.6 | 44 |
| Ring analysis ASTM D3238 | | | | | | |
| %CA | 0 | 0 | 0 | 0 | 0 | 0 |
| %CN | 7.9 | 12 | 9.2 | 21.8 | 22.9 | 31.2 |
| %CP | 92.1 | 88 | 90.8 | 78.2 | 77.1 | 68.8 |
| Sulphur content mass% ASTM D2622 | <0.01 | <0.01 | 3.3 | 2.75 | 4 | 2.5 |
| Flash point (CCC) °C JIS K2265-4 | 220 | 3.45 | 204 | 220 | 256 | 194 |
| Pour point °C JIS K 2269 | -37.5 | 3.8 | -37.5 | 2.1 | -12.5 | -32.5 |

The aforementioned raw materials were blended as shown in Tables 2 and 3, and the lubricating oil compositions of Examples of Embodiment 1 to 8 and Comparative Examples 1 to 10 were obtained.

### Evaluation

Next, evaluation tests were carried out in respect of the lubricating oil compositions of Examples of Embodiment 1 to 8 and Comparative Examples 1 to 10. It was confirmed that all the lubricating oil compositions for Examples of Embodiment 1 to 8 satisfied 5W-30.

An evaluation of the fuel consumption characteristics was carried out on the basis of fuel consumption bench tests using a 4000 cc diesel engine of Japanese make. The operating conditions were set up with reference to the Ministry of Land, Infrastructure and Transport 10•15 mode. The gallery temperature at measurement time was set at 90°C. The results shown in Tables 2 and 3 show the rate of improvement (%) in fuel economy when taking as a criterion a commercial diesel engine oil classified as SAE viscosity grade 10W-30. In the evaluation, if the rate of improvement (%) in fuel economy was at least 1.0, the fuel consumption characteristics were marked O (good).

The Noack volatility (%) was measured on the basis of ASTM D5800. For the evaluation, if the Noack volatility (%) was not more than 13.0, volatility was marked O (good).

Hot tube tests were carried out in accordance with the Japan Petroleum Institute's standard JPI-5S-55-99 "Engine oils - Hot tube test." The test conditions were set at a test temperature of 290°C/300°C, test duration 16 hours, sample oil feed rate of 0.3 ml/hour and air flow of 10 ml/hour, and if the evaluation (merit points) of the colour of discoloured portion of the glass tube after completion of the test was at least 7.0, detergency was marked O (good).

The [capillary viscosity - TBS viscosity) / TBS viscosity] was calculated by following the aforementioned method.

In addition, the (40°C) kinematic viscosity, (100°C) kinematic viscosity, viscosity index (VI), boron content (total value), calcium content (total value), phosphorus content (total value), zinc content (total value), nitrogen content (total value) and molybdenum content (total value) were calculated (the base stock Vk 100°C was the 100°C kinematic viscosity of the base oil mixture).

**Table 2- Inventive Examples**

| Example | 1 | 2 | 3 | 4 | 5 | 6 | 7 | 8 |
|---|---|---|---|---|---|---|---|---|
| Base oil 1 | 57.60 | 57.60 | 57.60 | 57.60 | 57.60 | 57.60 | 57.60 | 57.60 |
| Base oil 2 | 28.37 | 28.37 | 28.37 | 28.37 | 28.37 | 28.37 | 28.37 | 28.37 |
| DH2 DI package 1 | 14.00 | 14.00 | 14.00 | 14.00 | 14.00 | 14.00 | 14.00 | - |
| DH2 DI package 2 | - | - | - | - | - | - | - | 14.00 |
| VI imp. solution 1 (comb-like PMA) | 5.5 (3.30) | - | - | 3.3 (1.98) | 2.75 (1.65) | 4 (2.40) | 2.5 (1.50) | 5.5 (3.30) |
| VI imp. solution 2 (comb-like PMA) | - | 12.4 (4.96) | 3.45 (1.38) | | | | | |
| VI imp. solution 3 (non-comb-like PMA) | - | - | 3.8 (2.28) | - | 2.05 (1.23) | | | |
| VI imp. solution 4 (olefin copolymer) | - | - | - | 3.1 (0.39) | - | - | - | - |
| VI imp. solution 5 (styrene-diene copolymer) | | | | | | 4.7 (0.31) | 9.4 (0.61) | |
| Defoamer | 0.03 | 0.03 | 0.03 | 0.03 | 0.03 | 0.03 | 0.03 | 0.03 |
| Total | 100.0 | 100.0 | 100.0 | 100.0 | 100.0 | 100.0 | 100.0 | 100.0 |
| Fuel economy improvement ratio 60°C (%) | O | O | O | O | O | O | O | O |
| Volatility NOACK | O | O | O | O | O | O | O | O |
| Detergency HTT (300°C) | O | O | O | O | O | O | O | O |
| Vk40 mm²/s | 42.23 | 42.42 | 49.46 | 49.24 | 46.89 | 45.73 | 49.51 | 42.24 |
| Vk100 mm²/s | 10.43 | 11.00 | 10.46 | 10.51 | 10.45 | 10.34 | 10.24 | 10.45 |
| VI | 248 | 264 | 208 | 210 | 221 | 224 | 201 | 248 |
| Base stock Vk 100°C mm²/s | 5.0 | 5.0 | 5.0 | 5.0 | 5.0 | 5.0 | 5.0 | 5.0 |
| (HTHS (capillary, 100°C)- HTHS (TBS, 100°C)/HTHS (TBS, 100°C) | 0.10 | 0.11 | 0.09 | 0.08 | 0.08 | 0.10 | 0.09 | 0.10 |
| B mass% | 0.033 | 0.033 | 0.033 | 0.033 | 0.033 | 0.033 | 0.033 | 0.027 |
| Ca mass% | 0.220 | 0.220 | 0.220 | 0.220 | 0.220 | 0.220 | 0.220 | 0.220 |
| P mass% | 0.096 | 0.096 | 0.096 | 0.096 | 0.096 | 0.096 | 0.096 | 0.096 |
| Zn mass% | 0.110 | 0.110 | 0.110 | 0.110 | 0.110 | 0.110 | 0.110 | 0.110 |
| N mass% | 0.120 | 0.120 | 0.120 | 0.120 | 0.120 | 0.120 | 0.120 | 0.120 |
| Mo mass% | <0.001 | <0.001 | <0.001 | <0.001 | <0.001 | <0.001 | <0.001 | <0.001 |
| Fuel efficiency test, oil temp. 60°C | | | | | | | | |
| FE improvement ratio against 10W-30 DH-2 oil % | 1.5 | 1.5 | 1.4 | 1.0 | 1.3 | 1.3 | 1.1 | 1.5 |
| NOACK % | 10.0 | 10.3 | 10.2 | 10.0 | 10.0 | 10.01 | 10.04 | 10.0 |
| Hot tube 290°C merit point | 8.0 | 8.0 | 8.0 | 8.0 | 8.0 | 8.0 | 8.0 | 8.0 |
| Hot tube 300°C merit point | 8.0 | 8.0 | 8.0 | 8.0 | 8.0 | 8.0 | 8.0 | 8.0 |

| | | | | | | | | |
|---|---|---|---|---|---|---|---|---|
| Note: Figures in brackets are polymer amounts minus diluents. | | | | | | | | |

**Table 3 - Comparative Examples**

| Comparative Example | 1 | 2 | 3 | 4 | 5 | 6 | 7 | 8 | 9 | 10 |
|---|---|---|---|---|---|---|---|---|---|---|
| Base oil 1 | | 57.60 | 57.60 | 57.60 | 57.60 | 24.80 | 79.36 | | | 57.60 |
| Base oil 2 | 84.43 | 28.37 | 28.37 | 28.37 | 28.37 | 57.87 | | | | 28.37 |
| Base oil 3 | | | | | | | | 76.47 | | |
| Base oil 4 | | | | | | | | | 63.39 | |
| Base oil 5 | | | | | | | | | 17.88 | |
| DH2 DI package 1 | 14.00 | 14.00 | 14.00 | 14.00 | 14.00 | 14.00 | 14.00 | 14.00 | 14.00 | |
| DH2 DI package 2 | | | | | | | | | | |
| DH2 DI package 3 | | | | | | | | | | 14.00 |
| VI imp. solution 1 (comb-like PMA) | 1.54 (0.92) | | | | | 3.3 (1.96) | 6.61 (3.97) | 9.5 (5.70) | 4.7 (2.82) | 5.5 (3.30 ) |
| VI imp. solution 2 (comb-like PMA) | | | | | | | | | | |
| VI imp. solution 3 (non-comb-like PMA) | | 5.1 (3.10) | | 3.8 (2.28) | | | | | | |
| VI imp. solution 4 (olefin copolymer) | | | 7.6 (0.95) | 2.3 (0.29) | | | | | | |
| VI imp. | | | | | 18.5 | | | | | |
| solution 5 (styrene-diene copolymer) | | | | | (1.20) | | | | | |
| Defoamer | 0.03 | 0.03 | 0.03 | 0.03 | 0.03 | 0.03 | 0.03 | 0.03 | 0.03 | 0.03 |
| Total | 100.0 | 100.0 | 100.0 | 100.0 | 100.0 | 100.0 | 100.0 | 100.0 | 100.0 | 100.0 |
| Fuel economy characteristics | | | | | | | | | | |
| FE improvement ratio 60°C (%) | X | X | X | X | X | X | O | O | O | O |
| Volatility NOACK | O | O | O | O | O | O | X | X | X | O |
| Detergency HTT (300°C) | O | O | O | O | O | O | O | O | O | X |
| Vk40 mm²/s | 61.49 | 51.91 | 58.97 | 53.70 | 58.35 | 52.85 | 38.52 | 33.41 | 44.28 | 42.30 |
| Vk100 mm²/s | 10.48 | 10.49 | 10.42 | 10.53 | 10.56 | 10.49 | 10.51 | 10.71 | 10.48 | 10.46 |
| VI | 160 | 197 | 167 | 190 | 173 | 193 | 278 | 332 | 237 | 249 |
| Base stock Vk 100°C mm²/s | 7.5 | 5.0 | 5.0 | 5.0 | 5.0 | 6.0 | 4.0 | 2.7 | 5.0 | 5.0 |
| (HTHS (capillary, 100°C)- HTHS (TBS, 100°C)/ HTHS (TBS, 100°C) | 0.03 | 0.06 | 0.06 | 0.06 | 0.06 | 0.06 | 0.17 | 0.19 | 0.10 | 0.10 |
| B mass% | 0.033 | 0.033 | 0.033 | 0.033 | 0.033 | 0.033 | 0.033 | 0.033 | 0.033 | 0.020 |
| Ca mass% | 0.220 | 0.220 | 0.220 | 0.220 | 0.220 | 0.220 | 0.220 | 0.220 | 0.220 | 0.220 |
| P mass% | 0.096 | 0.096 | 0.096 | 0.096 | 0.096 | 0.096 | 0.096 | 0.096 | 0.096 | 0.096 |
| Zn mass% | 0.110 | 0.110 | 0.110 | 0.110 | 0.110 | 0.110 | 0.110 | 0.110 | 0.110 | 0.110 |
| N mass% | 0.120 | 0.120 | 0.120 | 0.120 | 0.120 | 0.120 | 0.120 | 0.120 | 0.120 | 0.100 |
| Mo mass% | <0.001 | <0.001 | <0.001 | <0.001 | <0.001 | <0.001 | <0.001 | <0.001 | <0.001 | <0.00 1 |
| Fuel efficiency test, oil temp. 60°C | | | | | | | | | | |
| FE improvement ratio against 10W-30 DH-2 oil % | -0.7 | 0.8 | 0.7 | 0.7 | 0.7 | 0.9 | 2.7 | 3.7 | 1.0 | 1.5 |
| NOACK % | 5.1 | 9.8 | 10.1 | 10.1 | 11.2 | 8.0 | 14.0 | 42.0 | 13.3 | 10.3 |
| Hot tube 290°C merit point | 8.0 | 8.0 | 8.0 | 8.0 | 8.0 | 8.0 | 8.0 | 8.0 | 8.0 | 8.0 |
| Hot tube 300°C merit point | 8.0 | 8.0 | 8.0 | 8.0 | 8.0 | 8.0 | 8.0 | 8.0 | 8.0 | 0.5 |

| | | | | | | | | | | |
|---|---|---|---|---|---|---|---|---|---|---|
| Note: Figures in brackets are polymer amounts minus diluents. | | | | | | | | | | |

## Claims

1. Lubricating oil composition for diesel engines **characterised in that** it contains:
a) a base oil with a kinematic viscosity at 100°C of 4.5 to 5.5 mm²/s, consisting of either a single GTL base oil with a kinematic viscosity at 100°C of 4.5 to 5.5 mm²/s or a mixture of i)a GTL base oil with a kinematic viscosity at 100°C of 3.0 to 6.0 mm²/s; and ii) a GTL base oil with a kinematic viscosity at 100°C of 7.0 to 13 mm²/s,
b) a comb-like polymethacrylate based viscosity index improver and
c) a boron-containing dispersant and boron-containing detergent, wherein the total amount of boron-containing dispersant and/or boron-containing detergent incorporated in terms of conversion to boron content relative to the total amount of the composition being not less than 0.025 mass% and not more than 0.050 mass%,
and wherein it satisfies 0W-30 or 5W-30 in the SAE J300 standard.

2. Lubricating oil composition for diesel engines in accordance with Claim 1 which includes a non-comb-like polymethacrylate based viscosity index improver and a styrene-diene copolymer based viscosity index improver and/or an olefin copolymer based viscosity index improver, and which further satisfies at least one of the following (1) to (3).
(1) Non-comb-like PMA based viscosity index improver content/total viscosity index improver content: not more than 0.7
(2) OCP based viscosity index improver content/total viscosity index improver content: not more than 0.2
(3) SCP based viscosity index improver content/total viscosity index improver content: not more than 0.3

3. Lubricating oil composition for diesel engines in accordance with Claim 1 or 2 satisfying the following viscosity characteristic: $\frac{\left[\begin{matrix}HTHS 100 ° C viscosity \left(capillary method\right) - \\ HTHS 100 ° C viscosity \left(TBS method\right)\end{matrix}\right]}{HTHS 100 ° C viscosity \left(TBS method\right)} = 0.07 to 0.15$ wherein HTHS 100°C viscosity (capillary method) is measured according to ASTM D5481 test method and the HTHS 100°C viscosity (TBS method) is measured according to ASTM D4683.

## Patentansprüche

1. Schmierölzusammensetzung für Dieselmotoren, **dadurch gekennzeichnet, dass** sie Folgendes enthält:
a) ein Grundöl mit einer kinematischen Viskosität bei 100 °C von 4,5 bis 5,5 mm²/s, das entweder aus einem einzelnen GTL-Grundöl mit einer kinematischen Viskosität bei 100 °C von 4,5 bis 5,5 mm²/s oder aus einer Mischung von i) einem GTL-Grundöl mit einer kinematischen Viskosität bei 100 °C von 3,0 bis 6,0 mm²/s; und ii) einem GTL-Grundöl mit einer kinematischen Viskosität bei 100 °C von 7,0 bis 13 mm²/s besteht,
b) einen kammartigen Viskositätsindexverbesserer auf Polymethacrylatbasis und
c) ein borhaltiges Dispergiermittel und ein borhaltiges Detergens, wobei die Gesamtmenge an integriertem borhaltigem Dispergiermittel und/oder borhaltigem Detergens bezüglich einer Umwandlung in einen Borgehalt relativ zu der Gesamtmenge der Zusammensetzung nicht weniger als 0,025 Masse-% und nicht mehr als 0,050 Masse-% beträgt,
und wobei es 0W-30 oder 5W-30 in dem SAE J300-Standard erfüllt.

2. Schmierölzusammensetzung für Dieselmotoren nach Anspruch 1, die einen nicht-kammartigen Viskositätsindexverbesserer auf Polymethacrylatbasis und einen Viskositätsindexverbesserer auf Styrol-Dien-Copolymerbasis und/oder einen Viskositätsindexverbesserer auf Olefincopolymerbasis beinhaltet und die ferner wenigstens einen der folgenden Punkte (1) bis (3) erfüllt.
(1) Gehalt an nicht-kammähnlichem Viskositätsindexverbesserer auf PMA-Basis/Gesamtgehalt an Viskositätsindexverbesserer: nicht mehr als 0,7
(2) Gehalt an Viskositätsindexverbesserer auf OCP-Basis/Gesamtgehalt an Viskositätsindexverbesserer: nicht mehr als 0,2
(3) Gehalt an Viskositätsindexverbesserer auf SCP-Basis/Gesamtgehalt an Viskositätsindexverbesserer: nicht mehr als 0,3

3. Schmierölzusammensetzung für Dieselmotoren nach Anspruch 1 oder 2, die die folgende Viskositätskenngröße erfüllt: $\frac{\left[\begin{matrix}HTHS - V i s k o s i t ä t bei 100 ° C \left(Kapillarver fahren\right) - \\ HTHS - V i s k o s i t ä t bei 100 ° C \left(TBS-Verfahren\right)\end{matrix}\right]}{HTHS - V i s k o s i t ä t bei 100 ° C \left(TBS-Verfahren\right)} = 0,07 bis 0,15$ wobei die HTHS-Viskosität bei 100 °C (Kapillarverfahren) gemäß einem ASTM D5481-Testverfahren und die HTHS-Viskosität bei 100 °C (TBS-Verfahren) gemäß ASTM D4683 gemessen wird.

## Revendications

1. Composition d'huile lubrifiante pour moteurs diesel **caractérisée en ce qu'**elle contient :
a) une huile de base avec une viscosité cinématique à 100 °C de 4,5 à 5,5 mm²/s, constituée soit par une seule huile de base GTL avec une viscosité cinématique à 100 °C de 4,5 à 5,5 mm²/s, soit par un mélange i) d'une huile de base GTL avec une viscosité cinématique à 100 °C de 3,0 à 6,0 mm²/s ; et ii) d'une huile de base GTL avec une viscosité cinématique à 100 °C de 7,0 à 13 mm²/s,
b) un agent améliorant l'indice de viscosité à base de polyméthacrylate en forme de peigne et
c) un dispersant contenant du bore et un détergent contenant du bore, la quantité totale de dispersant contenant du bore et/ou de détergent contenant du bore incorporée en termes de conversion en teneur en bore par rapport à la quantité totale de la composition n'étant pas inférieure à 0,025 % en masse et pas supérieure à 0,050 % en masse, et la composition satisfaisant 0W-30 ou 5W-30 suivant la norme SAE J300.

2. Composition d'huile lubrifiante pour moteurs diesel selon la revendication 1, qui comporte un agent améliorant l'indice de viscosité à base de polyméthacrylate n'étant pas en forme de peigne et un agent améliorant l'indice de viscosité à base de copolymère de styrène-diène et/ou un agent améliorant l'indice de viscosité à base de copolymère d'oléfine, et qui satisfait en outre au moins l'une des caractéristiques (1) à (3) suivantes.
(1) teneur en agent améliorant l'indice de viscosité à base de PMA n'étant pas en forme de peigne/teneur totale en agent améliorant l'indice de viscosité : pas plus de 0,7
(2) teneur en agent améliorant l'indice de viscosité à base d'OCP/teneur totale en agent améliorant l'indice de viscosité : pas plus de 0,2
(3) teneur en agent améliorant l'indice de viscosité à base de SCP/teneur totale en agent améliorant l'indice de viscosité : pas plus de 0,3

3. Composition d'huile lubrifiante pour moteurs diesel selon la revendication 1 ou 2 satisfaisant la caractéristique de viscosité suivante : $\frac{\left[\begin{matrix}Viscosit é HTHS à 100 ° C \left(methodé capillaire\right) - \\ viscosit é HTHS à 100 ° C \left(methodé TBS\right)\end{matrix}\right]}{v i s c o s i t é HTHS à 100 ° C \left(methodé TBS\right)} = 0,07 à 0,15$ la viscosité HTHS à 100 °C (méthode capillaire) étant mesurée selon la méthode d'essai ASTM D5481 et la viscosité HTHS à 100 °C (méthode TBS) étant mesurée selon la méthode d'essai ASTM D4683.
